

## UNITED STATES PATENT OFFICE.

CARL PIERCE LEWIS, OF SAN FRANCISCO, CALIFORNIA, ASSIGNOR TO MINERALS SEPARATION NORTH AMERICAN CORPORATION, OF NEW YORK, N. Y., A CORPORATION OF MARYLAND.

## ORE CONCENTRATION.

No Drawing.

Application filed July 26, 1920. Serial No. 399,008.

*To all whom it may concern:*

Be it known that I, CARL PIERCE LEWIS, a citizen of the United States, residing at San Francisco, State of California, have invented certain new and useful Improvements in Ore Concentration, of which the following is a specification.

This invention relates to ore concentration and is herein disclosed as especially applied to the selective froth-flotation separation of more or less complex ores, with the production of a concentrate, or separate concentrates, relatively rich in the desired minerals, and relatively free from the undesirable minerals. It will, however, appear that the flotation agents herein disclosed may be applied to collective flotation.

Ores which contain certain metals such as zinc, and more especially those which contain lead and zinc, together with iron and perhaps other values, have hitherto been found difficult ores to concentrate in forms that made satisfactory products for the smelter. Even in many cases where the ores were comparatively rich, it has been found difficult to satisfactorily separate such metals as the lead and zinc constituents sufficiently from each other and from the normally-floatable iron, if present, to enable the ores to be profitably worked. This has often been the case with lead-zinc ore even though the lead was present as galena, the zinc was present as blende, and the iron was present as pyrite.

I have discovered that with a flotation agent such as crude solvent naphtha or certain oils derived from coal tar, concentrates may be obtained in much more merchantable or smelterable form, especially in freedom from iron, than has hitherto been possible. I have found that iron-bearing ores of copper and the precious metals may also be made to yield concentrates remarkably free from iron if concentrated with such agents. I have found that xylene is a highly effective constituent of the flotation agents mentioned, especially when it carried naphthalene in solution, as it did in the coal tar oil used. Moreover, certain mixtures of benzene-series hydrocarbons have been found more effective than individual benzene-series hydrocarbons, especially when

carrying, in admixture or solution, naphthalene or certain naphthalene derivatives.

By adjusting the amount of hydrocarbons or mixtures used I have, for example, been able to effect a remarkably complete recovery of zinc singularly free from iron, thus greatly enhancing the value of the concentrate. I have also discovered that when such a hydrocarbon, especially a xylene containing naphthalene or certain other heavy hydrocarbons is used as a froth-flotation agent in small amounts on such ores, say around three-quarters of a pound to a pound and a half per ton of ore, a concentrate rich in lead and poor in zinc and iron may be obtained; and the tailings from this treatment, with the addition of another similar or smaller quantity of such hydrocarbon, even omitting the naphthalene ingredient, can be concentrated to recover an extraordinarily large proportion of the zinc comparatively free from lead and iron. Working in this way the recovery of lead may often be substantially improved and obtained at lower cost partly owing to the relative low price of naphthalene. The presence of the naphthalene and a benzene-series hydrocarbon in the tailings from the lead treatment in no way interferes with, and sometimes appears to facilitate, the clean recovery of a relatively large proportion of zinc.

I have found that benzene itself is not as efficient as the higher members of the series under most conditions. A mixture of the heavier hydrocarbons of this series, such as is sold under the name of solvent naphtha, is usually more efficient than would be supposed from a comparison of the results obtained by using the pure hydrocarbons higher up in the series. In effecting the concentration of lead and zinc in the manner described, there is often also effected a very complete recovery of gold and silver, variously divided among the concentrates, and the same is true of copper.

I have discovered that anthracene may be used instead of naphthalene. Anthracene differs from naphthalene in containing three benzene nuclei instead of the two benzene nuclei in naphthalene.

Naphthalene or the benzene series hydro-

carbons may be used in connection with a small amount of other frothing agent, such as pine oil. Naphthalene dissolved in pine oil confers on the solution some selective powers, but owing to the necessary predominance of the pine oil in such a solution, the selective effect of the naphthalene is somewhat masked in the absence of benzene-series hydrocarbon, or its equivalent. It will be observed that naphthalene may be used in solution as a collective frothing agent when it is not desired to effect selective collection of minerals.

A solution of naphthalene in Squibb's liquid petrolatum (sold as containing upwards of 99% napthenes) has substantially the advantages of a xylene solution of naphthalene.

Phenol and the cresols are less satisfactory since I find that they tend to cause a collective float, i. e., they fail to reject the iron pyrites.

It should be noted in connection with all the above named aromatic series flotation agents that one of their remarkable characteristics is their non-interference with selection of zinc over iron if used for the selection of lead prior to the flotation of the zinc.

In a number of tests a thousand grams of the ore were ground in a laboratory ball mill at normal temperature making a one to one pulp. As a rule eighty mesh grinding was found sufficient. The pulp placed in a laboratory flotation machine of the subaeration type and diluted with tap water to make a pulp of 3.5 parts water to one of ore, was then agitated slowly (say at a peripheral speed of 900 feet per minute) while a saturated solution of naphthalene in xylene was added to the pulp at the rate of 0.8 pounds per ton of ore treated. This mixture was then agitated at full speed, that is, at 1700 peripheral feet per minute for a two-minute period, after which opening the air port introduced air, with the formation of a mineral-bearing froth, which was removed during a ten-minute period, after which time very little froth formed. A spitzkasten machine on a number of ores gave similar results. Heating the pulp often improved the selection and the recovery.

The concentrate thus produced from Gnome Mining Co. lead-zinc ore was 9.0% of the original weight, and assayed as follows:

|        | Assay.    | % of original. |
|--------|-----------|----------------|
| Silver | 18.05 oz. | 62.6           |
| Lead   | 60.4%     | 91.0           |
| Zinc   | 7.5       | 16.0           |
| Copper | 2.94      | 49.4           |
| Iron   | 4.3       | 8.8            |
| Insol  | 5.3       |                |

To the remaining pulp were then added 65 2.3 pounds per ton of xylene. This mixture was given agitation at full speed for a two minute period, after which air was introduced to the pulp and the operation continued and the froth removed. The concentrate, when assayed, was found to be 11.1% of the original weight and to contain the following:

|        | Assay.   | % of original. | 75 |
|--------|----------|----------------|----|
| Silver | 6.32 oz. | 27.4           |    |
| Lead   | 4.8%     | 9.0            |    |
| Zinc   | 29.8%    | 80.2           |    |
| Copper | 2.0%     | 41.6           |    |
| Iron   | 9.0%     | 23.0           | 80 |

The tailings contained 68.2% of the iron but only 10% of the silver, 9% of the copper, 3.8% of the zinc and no lead.

To obtain a further concentration the lead concentrate obtained as above described was placed in the machine while 1.3 pounds per ton (of the weight of original ore) of a saturated solution of naphthalene in xylene were added together with tap water at normal temperature to fill the machine to the proper level; meanwhile being slowly agitated. After two minutes agitation at full speed, air was introduced to the pulp and as the operation continued, a mineral bearing froth was removed. This cleaner concentrate constituted 6.4% of the original ore and on assay was found to contain the following:

|        | Assay.    | % of original. | 80 |
|--------|-----------|----------------|----|
| Silver | 17.20 oz. | 42.5           |    |
| Lead   | 69.8 %    | 73.5           |    |
| Zinc   | 6.6 %     | 10.0           |    |
| Copper | 2.08%     | 24.8           |    |
| Iron   | 3.0 %     | 4.4            | 80 |
| Insol  | 1.0 %     |                |    |

The residual pulp constituted the lead middling and was removed. Its assay was as follows:

|        | Assay.    | % of original. | 810 |
|--------|-----------|----------------|-----|
| Silver | 20.10 oz. | 20.1           |     |
| Lead   | 41.0 %    | 17.5           |     |
| Zinc   | 9.6 %     | 6.0            |     |
| Copper | 5.08%     | 24.6           |     |
| Iron   | 7.4 %     | 4.4            | 815 |
| Insol  | 16.0 %    |                |     |

The zinc concentrate obtained as above described was placed in the machine and agitated slowly while 1.5 pounds per ton (of the weight of original ore) of xylene was added with sufficient tap water at normal temperature to fill the machine to the proper level. This was then agitated at full speed for a two minute period after which air was introduced and the operation continued and a froth removed. This product constituted

the finished zinc concentrate constituting 6.5% of the weight of the original ore and was found to assay as follows:

|        | Assay.   | % of original. |
|--------|----------|----------------|
| Silver | 7.71 oz. | 19.7           |
| Lead   | 6.6 %    | 7.2            |
| Zinc   | 46.4 %   | 73.7           |
| Copper | 2.80 %   | 34.5           |
| Iron   | 7.5 %    | 11.3           |
| Insol  | 2.4 %    |                |

The residual pulp constituted the zinc middling, amounting to 4.6% of the original ore, and assayed as follows:

|        | Assay.   | % of original. |
|--------|----------|----------------|
| Silver | 4.31 oz. | 7.7            |
| Lead   | 2.3 %    | 1.8            |
| Zinc   | 5.8 %    | 6.5            |
| Copper | .84 %    | 7.1            |
| Iron   | 11.2 %   | 11.7           |

Bluff & Fairview mixed ores of the Britannia Mining Company gave the recoveries summarized below when treated analogously as follows: Treatment A (to produce rougher copper concentrates) carbonate of soda 8 pounds and saturated solution of naphthalene in xylene 1.2 per ton, froth removed during 8 minutes. Retreatment A (to produce cleaner copper concentrates "A", and middlings "A") 0.4 lbs. per ton of same xylene solution, froth removed during 5 minutes. Treatment B (to produce rougher zinc concentrates) 1.8 lbs. xylene per ton, froth removed during 14 minutes. Retreatment B (to produce cleaner zinc concentrates "B" and middlings "B") 0.7 lbs. xylene per ton, froth removed during 12 minutes.

|            | Assay. |       |      |      | % recovery. |       |       |
|------------|--------|-------|------|------|-------------|-------|-------|
|            | Wt. %  | Cu.   | Zn.  | Fe.  | Cu.         | Zn.   | Fe.   |
| Heads      | 100.0  | 2.35  | 4.6  | 12.8 | 100.0       | 100.0 | 100.0 |
| Conc. "A"  | 9.3    | 19.92 | 14.8 | 25.0 | 78.8        | 29.4  | 18.2  |
| Midds. "A" | 6.8    | 4.60  | 15.8 | 34.8 | 13.3        | 22.9  | 18.6  |
| Conc. "B"  | 3.3    | 1.44  | 59.8 | 2.0  | 2.0         | 42.4  | 5     |
| Midds. "B" | 1.6    | 1.72  | 15.0 | 15.4 | 1.2         | 5.3   | 2.0   |
| Tailing    | 79.0   | .14   | No.  | 9.8  | 4.7         | ----- | 60.7  |

A treatment of the San Francisco Del Oro ore of Mexico analogous to Gnome ore with 1.6 lbs. concentrated solution of naphthalene in xylene and 8.0 lbs. carbonate of soda per ton, yielded a lead concentrate containing 59.8% lead, 11.4% zinc, and 3.7% iron; recovering 78% of the lead. A further treatment of the residual pulp with 1.8 lbs. xylene per ton of original ore yielded a zinc concentrate containing 45.2% zinc, 4.9% lead, and 9% iron, recovering 81.2% of the zinc.

A similar two-stage treatment of ore from the Golconda Mine at Kingman, Arizona, of

the Highland Mining and Milling Company, similar to the Gnome ore, but using sodium sulphide at the rate of 3 lbs. per ton of ore, worked out as follows, neglecting the trace of lead:

|           | Wt. % | Au.  | Ag.  | Cu.  | Zn.  | Fe.  |  |
|-----------|-------|------|------|------|------|------|--|
| Heads     | 100.0 | .05  | 9.50 | .63  | 12.5 | 8.8  |  |
| Conc. "A" | 10.3  | 0.19 | 35.0 | 3.20 | 7.6  | 31.2 |  |
| Conc. "B" | 23.3  | 0.10 | 21.6 | 1.12 | 44.8 | 6.8  |  |
| Tails     | 66.4  | .01  | 1.3  | .06  | 1.8  | 6.0  |  |

|           | Au.   | Ag.   | Cu.   | Zn.   | Fe.   |    |
|-----------|-------|-------|-------|-------|-------|----|
| Heads     | 100.0 | 100.0 | 100.0 | 100.0 | 100.0 |    |
| Conc. "A" | 39.7  | 38.2  | 52.4  | 6.3   | 36.7  |    |
| Conc. "B" | 46.9  | 52.8  | 41.3  | 84.1  | 17.9  |    |
| Tails     | 13.4  | 9.0   | 6.3   | 9.6   | 45.4  | 85 |

Simon silver-lead ore of Mina, Nevada, when concentrated first with soda ash 3 lbs. per ton and a solution of anthracene in solvent naphtha 0.6 lbs. per ton yielded a lead concentrate in a froth collected for a period of six minutes. Treatment of the remaining pulp with 1.6 lbs. per ton of crude solvent naphtha yielded a zinc concentrate in a froth collected for twenty minutes. The concentrates were not retreated. A subaeration laboratory machine was used at normal temperature. The results are summarized below:

|           | % Wt. | Oz. Ag. | % Pb. | % Zn. | % Fe. | % Insol |  |
|-----------|-------|---------|-------|-------|-------|---------|--|
| Feed      | 100.0 | 4.50    | 6.3   | 7.6   | 6.5   |         |  |
| Pb. Conc. | 7.9   | 35.72   | 63.1  | 5.6   | 2.7   | 11.2    |  |
| Zn. Conc. | 15.1  | 8.0     | 8.8   | 38.4  | 7.5   | 13.8    |  |
| Tails     | 77.0  | 0.6     | Tr.   | 1.8   | 6.7   |         |  |

|           | Ag.  | Pb.   | Zn.  | Fe.  |     |
|-----------|------|-------|------|------|-----|
| Feed      | 100. | 100.  | 100. | 100. |     |
| Pb. Conc. | 63.0 | 79.2  | 5.7  | 3.2  |     |
| Zn. Conc. | 26.9 | 20.8  | 76.3 | 17.4 | 115 |
| Tails     | 10.1 | ----- | 18.0 | 79.4 |     |

The ore of the Tomboy mine of Telluride, Colorado, gave better recoveries but with concentrates slightly less clean when subjected to three-stage treatment, followed by retreatment of the third concentrate; first (A) with five pounds of carbonate of soda and 0.2 pounds of methyl alcohol solution of naphthalene; second (B) with 0.2 pounds of the same naphthalene solution; third (C) with 0.7 pounds of heavy naphtha from coal tar, and retreatment of the third concen-

trate with 0.3 pounds of the same naphtha. The results are summarized below:

## Assays.

|              | % Wt. | Au.  | Ag.  | Cu.  | Pb.  | Zn.  | Fe.  |
|--------------|-------|------|------|------|------|------|------|
| Heads.....   | 100.0 | .097 | 1.87 | 1.16 | 4.6  | 5.4  | 6.4  |
| Conc. A..... | 6.5   | .19  | 14.3 | 7.60 | 47.6 | 6.4  | 12.0 |
| Conc. B..... | 4.5   | .39  | 10.5 | 8.00 | 18.4 | 22.0 | 15.4 |
| Conc. C..... | 8.6   | .50  | 4.8  | 2.30 | 7.6  | 44.0 | 11.1 |
| Midds.....   | 5.1   | .50  | 0.6  | .44  | 1.1  | 3.9  | 10.7 |
| Tails.....   | 75.3  | .005 | .08  | .11  | No.  | No.  | 3.5  |

## Recoveries.

|              | Au.   | Ag.   | Cu.   | Pb.   | Zn.   | Fe.   |
|--------------|-------|-------|-------|-------|-------|-------|
| Heads.....   | 100.0 | 100.0 | 100.0 | 100.0 | 100.0 | 100.0 |
| Conc. A..... | 12.1  | 49.0  | 42.7  | 66.8  | 7.6   | 12.0  |
| Conc. B..... | 17.2  | 24.7  | 31.1  | 17.9  | 18.3  | 10.7  |
| Conc. C..... | 42.2  | 21.6  | 17.1  | 14.0  | 70.4  | 14.7  |
| Midds.....   | 25.0  | 1.6   | 1.9   | 1.3   | 3.7   | 21.8  |
| Tails.....   | 3.5   | 3.1   | 7.2   | ----- | ----- | 40.8  |

Not only can the present invention be used to make possible the froth-flotation separation of ores hitherto considered commercially unworkable by flotation, such as the mixed lead, zinc and iron ores, but it improves the froth-flotation separation of other ores. Among other advantages it can easily be so operated as to keep the calcium fluoride content of concentrates well within the limits set by the smelters.

Ore of the Emma mine, at Eholt, British Columbia, made into a 3.5 to 1 pulp with tap water at normal temperature gave the following results:

## Assays.

|            | % Wt. | Au.  | Ag.  | Cu.   | Fe.  |
|------------|-------|------|------|-------|------|
| Heads..... | 100.  | .034 | .20  | .86   | 25.0 |
| Conc.....  | .6    | .43  | 3.43 | 10.13 | 25.7 |
| Tails..... | 92.4  | Tr.  | Tr.  | .09   | 24.8 |

## Recoveries.

|            | Au.   | Ag.   | Cu.   | Fe.   |
|------------|-------|-------|-------|-------|
| Heads..... | 100.0 | 100.0 | 100.0 | 100.0 |
| Conc.....  | 99.0  | 99.0  | 90.6  | 7.8   |
| Tails..... | 1.0   | 1.0   | 9.4   | 92.2  |

A spitzkasten machine was used, and the flotation agent, consisting of nine parts of a solution of naphthalene in crude solvent naphtha and one part of Pensacola #350, was used at the rate of 1.4 lbs. per ton of ore. The Pensacola #350 is a crude pine oil made by destructive distillation of wood.

Nevada Douglas Copper Company ore from Ludwig, Nevada, containing 3.16% copper and 13% iron when concentrated in a subaeration type laboratory testing machine using commercial crude solvent naphtha as a flotation agent, produced a concentrate containing 26.2% copper and 28 to 29% iron; recovering more than 90% of the

copper, while the tailings contained 60% of the iron.

Ore from the Le Roi mine, Rossland, British Columbia, containing .25 ounces of gold, 2.38% of copper, 30.7% iron, and 37.49% insoluble, when concentrated with 2.9 pounds per ton of Barret No. 1 oil mixed with .2 pounds per ton of crude pine oil yielded a concentrate containing 1.18 ounces gold, 12.96% copper, 35.4%, giving a recovery of 96.8% of gold, and 96.2% of copper. The tailings contained 78% of the original iron. When the pulp temperature was raised from its normal temperature of 50° F. to 90° F. the concentrates were richer and the separation more rapid.

The No. 1 oil was found to contain 15% of naphthalene on distillation.

The froth-flotation concentration of the Knob Hill ore of Republic, Washington, was effected in a single step, with a mixture containing solvent naphtha, nine parts, and one part of the crude pine oil, known as "Pensacola #350". The mixture was used at the rate of 1.2 lbs. per ton of ore.

The concentrates contained 99.9% of both the gold and the silver, and the tailings contained 78.1% of the iron.

A copper-iron ore from Sunlock Mining Co's. mine, Vancouver Island, B. C., treated similarly to the Knob Hill ore as above described produced a concentrate assaying 25% copper and containing 98% of the original copper.

Even such a refractory ore as Sullivan lead-zinc ore of Kimberley, B. C. gave excellent results when concentrated first with ten pounds of carbonate of soda and 0.8 lbs. of a saturated solution of naphthalene in xylene (both per ton of ore), and then concentrated with 1.6 lbs. xylene combined with 0.6 lbs. benzene, all as outlined above. The results are itemized below. The first portion of froth formed after the addition of the naphthalene solution was collected separately as a lead concentrate. The remainder of the same froth was collected as a lead middling. The froth following the addition of the benzene mixture was similarly collected as a zinc concentrate and a zinc middling.

|                | Assays. |      |      |      | % recovery. |       |       |
|----------------|---------|------|------|------|-------------|-------|-------|
|                | Wt. %   | Pb.  | Zn.  | Fe.  | Pb.         | Zn.   | Fe.   |
| Heads.....     | 100.0   | 12.3 | 17.9 | 29.4 | 100.0       | 100.0 | 100.0 |
| Pb. Concs..... | 11.1    | 60.0 | 8.0  | 9.8  | 54.4        | 5.0   | 3.7   |
| Pb. Midds..... | 6.0     | 50.2 | 15.5 | 9.0  | 24.3        | 5.1   | 1.6   |
| Zn. Concs..... | 22.4    | 5.0  | 50.6 | 9.8  | 9.1         | 63.2  | 7.5   |
| Zn. Midds..... | 7.8     | 9.2  | 34.0 | 18.8 | 5.6         | 14.7  | 5.0   |
| Tailings.....  | 52.7    | 1.5  | 4.1  | 45.6 | 6.4         | 12.0  | 81.0  |

The hitherto refractory Anaconda zinc ore gave remarkable results. The ore wet-ground to about 80 mesh, made into a 3.5 to

1 pulp with tap water at normal temperature, was subjected to froth-flotation in a subaeration machine, when mixed with 10 lbs. carbonate of soda and 0.4 lb. of a saturated solution of naphthalene in xylene per ton of ore. The froth removed for a period of seven minutes yielded the lead concentrate set forth below. To the remaining pulp was added 2.1 lbs. of crude solvent naphtha per ton of original ore and the zinc concentrate froth removed for a period of twenty-six minutes. No retreatments were made.

| 15        | Assays.  |            |          |          |          |          |        |
|-----------|----------|------------|----------|----------|----------|----------|--------|
|           | %<br>Wt. | Oz.<br>ag. | %<br>Cu. | %<br>Pb. | %<br>Zn. | %<br>Fe. | Insol. |
| 20 Heads  | 100      | 2.40       | .65      | 8.5      | 13.5     | 12.8     |        |
| Pb. Conc. | 9.0      | 4.56       | 2.60     | 58.5     | 11.5     | 4.1      | 70     |
| Zn. Conc. | 26.7     | 5.30       | 1.36     | 11.8     | 46.0     | 5.3      |        |
| Tailings  | 64.3     | 0.92       | 0.08     | 0.1      | 0.3      | 17.4     | 75     |

| 25        | Recoveries. |       |       |       |       |
|-----------|-------------|-------|-------|-------|-------|
|           | Ag.         | Cu.   | Pb.   | Zn.   | Fe.   |
| Heads     | 100.0       | 100.0 | 100.0 | 100.0 | 100.0 |
| Pb. Conc. | 17.2        | 36.2  | 62.3  | 7.7   | 2.8   |
| Zn. Conc. | 58.2        | 56.1  | 37.0  | 90.9  | 10.9  |
| Tailings  | 24.6        | 7.7   | 0.7   | 1.4   | 86.3  |

30 It will be noted that this complex pyrite lead-zinc ore given substantially the simplest treatment described above for lead-zinc ores, yielded concentrates suitable for commercial smelting, and of a grade and recovery hitherto unapproached. Attention is especially called to the low iron content of the concentrates, over 86% of the iron being discarded with the tailings.

40 The amounts of reagents set forth above are examples only and are subject to change to suit the needs of varying working conditions and of different ores. So also the working conditions, if any, will be adjusted to different ores. As is well known in the art the exact working conditions for best results in the treatment of any ore can only be determined in practice.

I claim:

50 1. The process of concentrating ores which consists in mixing with an ore pulp a flotation agent including a heavy hydrocarbon carried in a hydrocarbon of the benzene series and dependent upon the presence of a substantial amount of both kinds of hydrocarbon for froth-producing properties, and also bringing gaseous bubbles into contact with the solid particles in the ore pulp so as to produce a mineral-bearing froth carrying a large proportion of a mineral of the ore, and separating the froth.

60 2. The process of concentrating ores which consists in mixing with an ore pulp a mineral-frothing agent substantially dependent on the presence of a heavy hydrocarbon and

a benzene-series hydrocarbon in the absence of soapy material to produce a mineral-bearing froth, and also bringing gaseous bubbles into contact with the solid particles in the ore pulp so as to produce mineral-bearing froth, and separating the froth.

3. The process of concentrating ores which consists in mixing with an ore pulp a mineral-frothing agent substantially dependent on the presence of an aromatic compound containing a plurality of benzene nuclei carried in a benzene-series hydrocarbon in the absence of soapy material to produce a mineral-bearing froth, and also bringing gaseous bubbles into contact with the solid particles in the ore pulp so as to produce mineral-bearing froth, and separating the froth.

4. The process of concentrating ores which consists in mixing with an ore pulp a mineral-frothing agent substantially dependent on the presence of an aromatic hydrocarbon containing a plurality of benzene nuclei carried in a benzene-series hydrocarbon in the absence of soapy material to produce a mineral-bearing froth, and also bringing gaseous bubbles into contact with the solid particles in the ore pulp so as to produce mineral-bearing froth, and separating the froth.

5. The process of concentrating ores which consists in mixing with an ore pulp a mineral-frothing agent substantially dependent on the presence of an aromatic hydrocarbon containing a plurality of benzene nuclei carried in a liquid hydrocarbon of the benzene-series in the absence of soapy material to produce a mineral-bearing froth, and also bringing gaseous bubbles into contact with the solid particles in the ore pulp so as to produce mineral-bearing froth, and separating the froth.

6. A process of concentrating ores containing zinc and normally floatable iron which consists in mixing with a pulp of such an ore a small enough quantity of a mineral-frothing agent substantially dependent on the presence of a benzene-series hydrocarbon to produce a mineral-bearing froth selective of zinc over iron, and also bringing gaseous bubbles into contact with the solid particles in the ore pulp so as to produce a mineral-bearing froth carrying a relatively large proportion of the zinc and a relatively small proportion of the iron so as to obtain a concentrate relatively rich in zinc.

7. A process of concentrating ores containing zinc and normally floatable iron which consists in mixing with a pulp of such an ore a small enough quantity of a mineral-frothing agent substantially dependent on the presence of crude solvent coal-tar naphtha to produce a mineral-bearing froth selective of zinc over iron, and also bringing gaseous bubbles into contact with the solid particles in the ore pulp so as to produce a mineral-bearing froth carrying a relatively large

proportion of the zinc and a relatively small proportion of the iron so as to obtain a concentrate relatively rich in zinc.

8. A process of concentrating ores containing zinc and normally floatable iron which consists in mixing with a pulp of such an ore a small enough quantity of a mineral-frothing agent substantially dependent on the presence of a benzene-series hydrocarbon 70 carrying napthalene in solution to produce a mineral-bearing froth selective of zinc over iron, and also bringing gaseous bubbles into contact with the solid particles in the ore pulp so as to produce a mineral-bearing froth 75 carrying a relatively large proportion of the zinc and a relatively small proportion of the iron so as to obtain a concentrate relatively rich in zinc.

9. A process of concentrating complex 20 ores which consists in mixing with a pulp of such an ore a small enough quantity of a mineral-frothing agent substantially dependent on the presence of napthalene in 25 solution to produce a mineral-bearing froth, and also bringing gaseous bubbles into contact with the solid particles in the ore pulp so as to produce a mineral-bearing froth relatively rich in one constituent of the ore, separating the froth concentrate, mixing 30 with the remaining pulp benzene-series hydrocarbon material, bringing gaseous bubbles into contact with said remaining pulp so as to produce a second mineral-bearing froth relatively rich in a second constituent 35 of the ore, and separating the second froth.

10. A process of concentrating complex ores which consists in mixing with a pulp of such an ore a small enough quantity of a mineral-frothing agent substantially dependent on the presence of a benzene-series hydrocarbon having napthalene in solution to produce a mineral-bearing froth selective of zinc over iron, and also bringing gaseous bubbles into contact with the solid particles 45 in the ore pulp so as to produce a mineral-bearing froth relatively rich in one constituent of the ore, separating the froth concentrate, mixing with the remaining pulp a further amount of frothing agent, bringing 50 gaseous bubbles into contact with said remaining pulp so as to produce a second mineral-bearing froth relatively rich in a second constituent of the ore, and separating the second froth.

11. A process of concentrating ores containing three metals which consists in mixing with the pulp of such an ore a small enough quantity of a mineral-frothing agent substantially dependent on the presence of a benzene-series hydrocarbon to produce mineral-bearing froth selective of one metal over another, and also bringing gaseous bubbles into contact with the solid particles in the ore pulp so as to produce a mineral-bearing froth relatively rich in the first metal,

separating the froth, mixing with the remaining pulp a mineral-frothing agent substantially dependent on the presence of benzene-series hydrocarbon material to produce a mineral-bearing froth, also bringing gaseous bubbles into contact with the solid particles in the ore pulp so as to produce a mineral-bearing froth relatively rich in the second metal, and separating the froth relatively rich in the second metal to obtain a 75 second concentrate containing a relatively small proportion of the first and third metals.

12. A process of concentrating ores containing lead, zinc and normally floatable iron which consists in mixing with a pulp of such an ore a mineral-frothing agent substantially dependent on the presence of a benzene-series hydrocarbon to produce a mineral-bearing froth selective of lead over 80 zinc and iron, and also bringing gaseous bubbles into contact with the solid particles in the ore pulp so as to produce mineral-bearing froth relatively rich in lead, separating the froth, mixing with the remainder of the pulp a further amount of mineral-frothing agent substantially dependent on the presence of benzene-series hydro-carbon material to produce a mineral-bearing froth, and also bringing gaseous bubbles into contact with the solid particles in the ore pulp so as to produce mineral-bearing froth relatively rich in zinc, and separating the froth so as to obtain a relatively large proportion 85 of the zinc.

13. A process of concentrating ores containing lead, zinc and normally floatable iron which consists in mixing with a pulp of such an ore a mineral-frothing agent substantially dependent on the presence of crude solvent coal-tar naptha to produce a mineral-bearing froth selective of lead over zinc and iron and also bringing gaseous bubbles into contact with the solid particles in the ore pulp so as to produce mineral-bearing froth, 90 and also bringing gaseous bubbles into contact with the solid particles in the ore pulp so as to produce mineral-bearing froth relatively rich in zinc, and separating the froth so as to obtain a relatively large proportion 95 of the zinc.

14. A process of concentrating ores containing lead, zinc and normally floatable iron which consists in mixing with a pulp of such an ore a mineral-frothing agent substantially dependent on the presence of crude solvent naptha to produce a mineral-bearing froth, and also bringing gaseous bubbles into contact with the solid particles in the ore pulp so as to produce mineral-bearing froth relatively rich in lead, separating the froth, 100

mixing with the remainder of the pulp a further amount of mineral-frothing agent substantially dependent on the presence of benzene-series hydrocarbon material to produce a mineral-bearing froth, and also bringing gaseous bubbles into contact with the solid particles in the ore pulp so as to produce mineral-bearing froth relatively rich in zinc, and separating the froth so as to obtain a relatively large proportion of the zinc.

15. A process of concentrating ores containing lead, zinc and normally floatable iron which consists in mixing with a pulp of such an ore a mineral-frothing agent substantially dependent on the presence of benzene-series hydrocarbon material carrying napthalene in solution to produce a mineral-bearing froth, and also bringing gaseous bubbles into contact with the solid particles in the ore pulp so as to produce mineral-bearing froth relatively rich in lead, separating the froth, mixing with the remainder of the pulp a further amount of mineral-frothing agent substantially dependent on the presence of benzene-series hydrocarbon material to produce a mineral-bearing froth, and also bringing gaseous bubbles into contact with the solid particles in the ore pulp so as to produce mineral-bearing froth relatively rich in zinc, and separating the froth so as to obtain a relatively large proportion of the zinc.

16. A process of concentrating ores containing zinc and normally floatable iron which consists in mixing with a pulp of such an ore a small enough quantity of a mineral-frothing agent substantially dependent on the presence of a benzene-series hydrocarbon carrying a solid hydrocarbon to produce a mineral-bearing froth selective of zinc over iron and also bringing gaseous bubbles into contact with the solid particles in the ore pulp so as to produce a mineral-bearing froth carrying a relatively large proportion of the zinc and a relatively small proportion of the iron so as to obtain a concentrate relatively rich in zinc.

17. A process of concentrating complex

ores which consists in mixing with a pulp of such an ore a small enough quantity of a mineral-frothing agent substantially dependent on the presence of a solid hydrocarbon in solution to produce a mineral-bearing froth, and also bringing gaseous bubbles into contact with the solid particles in the ore pulp so as to produce a mineral-bearing froth relatively rich in one constituent of the ore, separating the froth concentrate, mixing with the remaining pulp benzene-series hydrocarbon material, bringing gaseous bubbles into contact with said remaining pulp so as to produce a second mineral-bearing froth relatively rich in a second constituent of the ore, and separating the second froth.

18. A process of concentrating complex ores which consists in mixing with a pulp of such an ore a small enough quantity of a mineral-frothing agent substantially dependent on the presence of a solid hydrocarbon dissolved in a volatile solvent to produce a mineral-bearing froth selective of one mineral constituent over another of the ore and also bringing gaseous bubbles into contact with the solid particles in the ore pulp so as to produce a mineral-bearing froth relatively rich in one constituent of the ore, separating the froth concentrate, mixing with the remaining pulp a further quantity of frothing agent, bringing gaseous bubbles into contact with said remaining pulp so as to produce a second mineral-bearing froth relatively rich in a second constituent of the ore, and separating the second froth.

19. The process of concentrating ores which consists in subjecting a pulp of the ore to froth-flotation separation with a mineral-frothing agent substantially dependent on the presence of crude solvent coal-tar naphtha in the absence of soapy material to produce a mineral-bearing froth, and separating the froth selective of a mineral of the ore.

In testimony whereof, I have affixed my signature to this specification.

CARL PIERCE LEWIS.